

July 27, 1937.

A. VON BIEHLER

2,088,145

LIGHT SENSITIVE MATERIAL

Filed Oct. 17, 1930

FIG. 1.



FIG. 2.



Inventor:

*Arpad von Biehler,*

By

Attorney

*Philip S. Hopkins.*

## UNITED STATES PATENT OFFICE

2,088,145

## LIGHT-SENSITIVE MATERIAL

Arpad von Biehler, Dessau in Anhalt, Germany,  
assignor to Agfa Anseco Corporation, Binghamton, N. Y., a corporation of New York

Application October 17, 1930, Serial No. 489,410  
In Germany October 23, 1929

4 Claims. (Cl. 95—9)

My present invention relates to a new photographic material and more particularly to photographic films having a stratified base which can be easily divided into some partial layers. One 5 of its objects is to provide a film coated on both sides with a photographic emulsion, wherein the film base can be split into two partial layer supports.

Another object of my invention is such a stratified film which can be separated into two partial layer supports and into a light filter.

Further objects of my invention will be seen from the detailed specification following hereafter.

15 It is known to make multi-color photographs by superposing in any order of succession several emulsion layers, sensitized for different spectral regions, and exposing them simultaneously behind an objective, if necessary with interposition of suitable filters. By this method, several colored partial negatives are obtained which are separated after exposure or development and are used for the preparation of a color positive. As 20 in this process it is of great importance that the several layers of emulsion should be in contact as nearly as possible while being exposed, proposals have already been made to apply two of the emulsion layers required on one and the same support. In the further course of the process, 25 one of said emulsion layers has to be stripped from the support and fixed on a new support. This requires, however, very intricate work and the thin emulsion pellicle is liable to be damaged.

30 According to my invention, this drawback is avoided by applying the sensitive layers one on each side of a support composed of one or more layers. Although the several strata of the layer support adhere firmly to one another they may 35 easily be separated, for example, by repeatedly sharply bending the support at one corner, into two supports each carrying a light-sensitive layer.

Of course, this detachable light-sensitive material may not only be used for the multi-color 40 photography but for all purposes requiring a material coated on both its sides with emulsion layers which are to be treated separately later on.

The support composed of several strata, may 45 consist of cellulose derivatives as well as of other suitable substances, such as artificial resins, rubber, and the like. The support may be composed either of several strata of the same material or of distinct materials of the same group, for instance, of several strata of different cellulose derivatives. Alternatively I may use for my com-

posite support strata of compounds belonging to different groups, for instance, two cellulose derivative strata and one rubber stratum. When superposing the different layers by casting, care must be taken that the strata can easily be disconnected. This can be attained by allowing the first stratum to dry completely before superposing the next stratum and by choosing the solvents of the casting solution to be applied in such a manner that they do not dissolve or swell the bottom stratum to a noticeable extent.

10 Besides, the different strata of the film base may contain any additions known in the manufacture of supports for photographic layers, for instance, pigments and dyestuffs. If it is necessary to optically separate the sensitive layers applied on each face of the support, one or several of the strata of the support may be suitably colored to constitute a color filter. If, when 15 printing, this color filter should be inconvenient, the base of the negative film may be built up in such a way that readily detachable strata are fitted, in the manner described, at both sides of the stratum containing the filter color, so that the support may be separated into three parts, 20 namely a filter layer and two supports each 25 carrying an emulsion layer.

In the following examples I illustrate in which manner the base of my new photographic films may be made.

30 *Example 1.*—From nitrocellulose dissolved in a mixture of 3 parts by volume of acetone and 2 parts by volume of methanol, a film is cast in the known manner. Then, onto this film, a layer of cellulose acetate is applied from an acetone 35 solution. When the latter is completely dried, finally, a second nitrocellulose film is cast thereon from a solution containing as a solvent a mixture of 3 parts by volume of ether and 1 part by volume of alcohol. The film base thus obtained, 40 shows two nitrocellulose strata enclosing a cellulose acetate stratum which strata firmly adhere together. However, the film base can be split between the upper nitrocellulose stratum and the cellulose acetate layer by repeatedly bending a 45 corner of it.

45 *Example 2.*—In an analogous manner, a film base may be made from cellulose acetate dissolved in acetone and of nitrocellulose dissolved in a solvent mixture containing ether and alcohol 50 in the ratio 3:1.

55 *Example 3.*—The film base may be composed of a nitrocellulose stratum cast from a solution containing ether and alcohol in the ratio 3:1, of a rubber layer cast from a rubber solution in 55

benzene and of a second nitrocellulose stratum, likewise, cast from a solution containing ether and alcohol in the ratio 3:1 and applied to the dried rubber layer.

5 My invention is not limited by the foregoing examples or by the specific details given therein. Thus, I may use, for instance, other cellulose derivatives or other solvents to prepare the casting solutions, care being taken, however, that 10 the said solvents do not act upon the stratum upon which they are cast. A few simple experiments should be made to determine the best kind of solvent or mixture of solvents to employ with a particular compound intended to form a 15 stratum of the composed film.

My new film bases may be coated either on one side or on both sides with a light-sensitive photographic emulsion in the known manner.

My invention is further illustrated by the accompanying drawing in which

Fig. 1 shows a film composed of two strata and

Fig. 2 a similar film comprising three strata.

In Fig. 1, A and B are two films consisting, for 25 instance, of the same or different cellulose derivatives or of other materials well known in the art as a film base. C and C' are the light-sensitive emulsions. The strata A and B adhering together, may be separated by detaching. Fig. 2 30 shows a similar film base comprising three detachable strata of which the middle D may be colored in order to provide a light filter.

The term "different cellulose derivatives" as used in the specification and the claims is intended to cover cellulose derivatives having differing solubility.

What I claim is:—

1. A photographic material comprising a strati-

fied support, the strata of which consist of at least two dry layers of differently soluble cellulose esters, said layers being fastened to each other over the whole surface solely by the adherence of the materials of the contacting layers, 5 whereby reduced adhesion of the layers is provided so that they are detachable by mechanical means.

2. A photographic material comprising a stratified support, the strata of which consist of at 10 least two dry layers of differently soluble cellulose esters, said layers being fastened to each other over the whole surface solely by the adherence of the materials of the contacting layers, 15 whereby reduced adhesion of the layers is provided so that they are detachable by mechanical means, and said stratified support being coated on at least one face with a light sensitive emulsion.

3. A photographic material comprising a stratified support the strata of which consist of a nitrocellulose layer and a cellulose acetate layer firmly adhering to each other to form one element and a nitrocellulose layer fastened to said cellulose acetate layer over the whole surface solely by 25 the adherence of the materials of the contacting layers, whereby reduced adhesion of the layers is provided, so that they are detachable by mechanical means.

4. A photographic material comprising a stratified support the strata of which consist of a nitrocellulose layer and a cellulose acetate layer fastened to said nitrocellulose layer over the whole surface solely by the adherence of the materials of the contacting layers, whereby reduced adhesion of the layers is provided so that they are 30 detachable by mechanical means.

ARPAD V. BIEHLER.